

## UNITED STATES PATENT OFFICE.

KARL DAEVES AND BRUNO WEISSENBERG, OF DUSSELDORF, GERMANY, ASSIGNORS TO THE FIRM: THYSSEN & CO., AKTIEN-GESELLSCHAFT, OF MULHEIM-RUHR, GERMANY.

METHOD OF MANUFACTURING HIGHLY-STRAINABLE IRON AND STEEL CONSTRUCTIONS.

No Drawing.

Application filed April 28, 1923. Serial No. 635,285.

To all whom it may concern:

Be it known that we, KARL DAEVES and BRUNO WEISSENBERG, citizens of the German Republic, and residing at Dusseldorf, 5 Germany, have invented certain new and useful Improvements in a Method of Manufacturing Highly-Strainable Iron and Steel Constructions, of which the following is a specification.

10 It is known to ascertain the reliability or safety of iron and steel constructions, particularly of pressure-reservoirs, by a testing-load. The magnitude of the latter can, however, be a limited one only, because 15 otherwise single parts of the construction are eventually strained beyond the yield-point and are liable to cold-deformation, and thereby, or by other reasons, the quality of the material is permanently influenced in 20 a detrimental way without the damages caused being after all perceptible. Thus, on the contrary to the purpose intended, the testing-load would result in endangering certain parts of the construction. Consequently, 25 the testing-load cannot be increased much above the actual working-pressure to be employed later on in practice.

It is further known that such changes of material and inner strains, for iron and 30 steel, can be completely overcome by a re-crystallization. The latter is attained by a short annealing within the limits of temperature at which the iron or steel are within the scope of solid solution. This temperature lies with pure iron above 900° centigrade and drops with increased carbon 35 contents down to 730° centigrade.

The improved method, according to the present invention, is based upon a combination 40 of corresponding working processes, and it is distinguished by the fact that the construction to be tested is, after its required connections—particularly weldings—are finished, exposed, first, to a testing-load up to the limit of the actually desired factor 45 of safety and, then, after said test to such an annealing that a re-crystallization takes place which removes the noxious result of

any overload caused by the test in the material of the construction.

The improved method is particularly adapted for testing the reliability or safety of weldings, especially of welded pressure-reservoirs such as, for instance, used for steam-boilers and the like.

Thereby, strainless steam-boilers can be manufactured, which are previously tested for pressures amounting to a multiple of the actual working-pressure at which the steam-boiler is used in practice.

Heretofore, such steam-boilers were exposed to a hydraulic test only, of which the pressure did not much exceed the actual working-pressure, according to the German steam-boiler law, for instance, for higher pressures 5 kgs. per cm.<sup>2</sup> only. Besides, in many such cases, it has been proved that just the overload occurring with hydraulic tests seriously endangered the material of the steam-boilers.

Likewise, a reliable manufacture of seamless reservoirs of high safety, of single constructional parts for bridges and buildings, of highly-trained parts of machinery such as pulleys, wheels, gearings and the like, is possible according to the improved method.

What we claim, is:—

A method of manufacturing highly-strainable iron and steel constructions consisting in exposing said constructions, first, to a testing-load up to the limit of the actually desired factor of safety and, then, after said test to such an annealing that a re-crystallization takes place which removes the noxious result of any overload caused by said test in the material of said constructions, substantially as set forth.

In testimony whereof we have hereunto set our hands in the presence of two subscribing witnesses.

KARL DAEVES.  
BRUNO WEISSENBERG.

Witnesses:

S. F. K. STEPHAN,  
D. ADOLF FRANK.